

## CEMENTED ZIRCONIUM BORIDE MATERIAL HAVING A PROTECTIVE CHROMIUM CONTAINING COATING

Frank W. Glaser, New York, N.Y., assignor, by mesne assignments, to Borolite Corporation, Pittsburgh, Pa., a corporation of Delaware

No Drawing. Application June 22, 1953  
Serial No. 363,376

2 Claims. (Cl. 117—118)

This application is a continuation-in-part of my application Serial No. 170,240, filed June 24, 1950.

This invention relates to shaped bodies of great strength at elevated temperatures which are resistant to corrosion and erosion in oxidizing or hot combustion gas atmospheres.

Shaped bodies of this invention are useful for gas turbine parts such as buckets, vanes and the like, of gas turbines, rocket nozzles, and the like, and for other purposes where operation at temperatures of about 700° C. and higher under corrosive conditions within an oxidizing atmosphere is involved.

In my co-pending application Serial No. 363,043, now abandoned, filed June 22, 1953, as a continuation-in-part of my said application Serial No. 170,240, now abandoned, there is disclosed and claimed a new hot strength corrosion-resisting structural material consisting of cemented zirconium diboride particles bonded by 2-7% of carbon-containing boron.

The present invention is based on the discovery that shaped articles of great hot-strength and corrosion-resistance at elevated temperatures for applications such as gas turbines, jet engines, and other applications of the foregoing type when made out of cemented particles of zirconium diboride  $ZrB_2$  which are bonded with about 2 to 7% boron containing in solid solution about 4 to 33 atomic percent carbon, although as such are superior to other known materials of this type heretofore used in or proposed for such applications, may be given a much greater life in hot corroding atmospheres by providing the exterior exposed surface layer of such body, with a surface stratum consisting of chromium oxide, chromium and boron, the chromium and boron being present in the surface stratum as dichromium boride  $Cr_2B$  with an excess of chromium. (Throughout this specification and claims, all proportions are given by weight unless otherwise specifically stated.)

In other words, the present invention is based on the discovery that shaped bodies formed of particles of  $ZrB_2$  that are bonded with 2 to 7% boron containing in solid solution about 4 to 33 atomic percent carbon, may be given considerably higher life in corrosive atmospheres if the exposed exterior of such body is provided with an integral protective surface layer which is substantially free of  $ZrB_2$  and contains essentially chromium oxide, chromium and boron, with the boron present principally as a part of a new compound dichromium boride  $Cr_2B$ .

A distinct feature of the invention is a shaped body having an exposed surface layer of particles of zirconium diboride  $ZrB_2$  bonded with 2 to 7 percent boron containing in solid solution about 4 to 33 atomic percent carbon, and having a surface stratum that is exposed to the hot corroding atmospheres, and which consists of chromium oxide, dichromium boride  $Cr_2B$ , and an excess of chromium, and which is substantially free of zirconium and zirconium diboride.

## Preparation of zirconium diboride powder

In one form of a satisfactory process of the invention amorphous boron in a form in which it is commercially available, zirconium hydride and carbon are used as the starting materials.

In order to obtain cemented zirconium diboride bodies of the invention having the desired high resistance to oxidation, corrosion and heat shock, it is essential that they shall be of a minimum purity of between 96.5 to 99% plus, i.e., that 96.5 to 99% plus of the cemented body shall consist of zirconium, boron and carbon only as  $ZrB_2$  with 2 to 7% carbon containing boron. It is important that the iron impurities be less than about 0.2% and preferably less than about 0.1%. It is also important to suppress and eliminate impurities of silicon carbide and other silicon impurities.

The zirconium and the zirconium hydride contains sometimes hafnium as an impurity, and such impurity may be present either in free or in solid solution with the cemented zirconium diboride  $ZrB_2$  which may also contain in solid solution minor impurities of other metals of the fourth group of the periodic system. These impurities may be present in amounts up to about 5% by weight without impairing the properties of the cemented zirconium diboride  $ZrB_2$  material to any appreciable extent with respect to oxidation, corrosion-resistance and shock resistance.

The mixture of the starting powder ingredients is compacted to reduce the powder volume, using dies and pressures of about  $\frac{1}{2}$  to 4 t.s.i., this pressure range having no critical significance. The powder mixture compacts are then placed into a graphite crucible which has a cover equipped with three stacks. One cover stack serves for the introduction of hydrogen into the crucible and another stack for burning the hydrogen leaving the crucible. The third stack serves for optical control of the temperature in the crucible. The crucible with the powder ingredient mixture contents is placed in a high frequency induction furnace, the crucible being provided with an insulating coating of lamp-black powder to reduce heat losses while being heated.

Before starting the heating, the interior of the crucible is purged with hydrogen and after purging, the hydrogen is ignited and the high frequency heating started while maintaining in the interior of the crucible, an atmosphere of hydrogen. Good results are obtained by induction heating with an alternating current of about 1000 to 3000 cycles per second. By way of example, with a powder mixture load of about 50 to 80 pounds held in a graphite crucible of 18 inches inside diameter, 4 feet height and 2 inches wall thickness, good results are obtained with an induction heater equipment capable of 60 kilowatt heating energy. Good results are obtained by heating with 40 to 50 kilowatts during the first 60 to 90 minutes of the heating cycle until the load is brought to a temperature of about 700 to 900° C. When this temperature is reached, the heat input is lowered since a relatively violent exothermic reaction takes place in the powder mixture as the zirconium diboride  $ZrB_2$  is being formed out of the powder ingredients at a temperature between about 1000 and 1200° C. Because of the heat developed at this stage of the process, by the exothermic reaction of the powder ingredients, the heat input should be reduced to prevent a too violent reaction that might damage the equipment and result in a loss of the production. By way of example, for a powder mixture load of about 50 pounds, the exothermic reaction lasts approximately 3 to 6 minutes, and the local heat generated during this period between the zirconium hydride and the boron of the powder mixture is estimated to be between about 2500 and 3500° C.

During the initial heating cycle at which the temperature of the powder mixture in the crucible is increased to about 900° C., there will take place a gradual decomposition of the zirconium hydride yielding continuously atomic hydrogen thereby providing the powder charge with a very effective additional protection. If zirconium powder in a form other than hydride is used in the starting powder mixture, the ultimate zirconium diboride obtained will be of somewhat lower purity.

Upon completion of the exothermic reaction, the full high frequency heating power of the induction heating equipment is applied to the crucible and there will be observed a relatively slow further rise of the temperature from about 1200° C. The slow temperature rise is due to the fact that the powder load has been greatly decreased by the formation of the zirconium diboride  $ZrB_2$  which has considerably higher heat conductivity than the original powder mixture in the crucible. It is desirable to have an additional heating cycle of about one hour with about 60 kilowatt heating energy in which the load is heated from 1200 to 1800° C., in order to eliminate impurities from the zirconium diboride  $ZrB_2$  that have been introduced by the use of impure boron in the original boron powder mixture. The principal boron impurity of the original powder consists of magnesium oxide which is reduced at temperatures about 1400° C. By heating the load to about 1800° C. with carbon originally introduced in the powder mixture or by the atmosphere of carbon oxide CO generated by the heated carbon crucible, the magnesium oxide will be reduced to magnesium metal which at temperatures between 1600 and 1800° C. will volatilize and leave or be expelled from the crucible, yielding a body of high purity zirconium diboride  $ZrB_2$  with the desired excess of 2 to 7% of carbon-containing boron.

The treated powder body should be maintained in the crucible at about 1800° C. for a period sufficient to eliminate all magnesium oxide and other volatile impurities present in the original powder mixture of ingredients. For loads of 10 to 75 pounds powder a treatment period of between 1 and 3 to 5 hours has been found satisfactory. In general, it is desirable to employ as the initial ingredient a grade of amorphous boron which contains the smallest amount of non-volatile impurities. It is very important that the iron impurities be less than 0.2% of the original boron of the mixture and that it should be substantially free from silicon carbide and other silicon impurities, it being desirable that the final powder produced shall contain 96.5 to plus 99% of the primary desired ingredients, to-wit, zirconium, boron and carbon in amounts corresponding to zirconium diboride  $ZrB_2$  with 2 to 7% boron, wherein the boron contains 4 to 33 atomic percent carbon in solid solution therewith.

Upon completion of the heating cycle at 1800° C. carried on in the manner described above, the crucible with its load is removed from the high frequency field and subjected to cooling for a time depending on the magnitude of the load. A hydrogen atmosphere should be maintained in the space in which the treated powder is cooled for at least 20 hours subsequent to completion of the heating cycle. In the example here considered, good results are obtained by passing the hydrogen at a rate of 5 cubic feet to 15 cubic feet per hour during the first 24 hours from the completion of the heating cycle and thereafter cooling with a flow of at about 5 cubic feet per hour. Excess hydrogen flow through the crucible during the cooling period will result in formation of water vapor at the burn-out region and will tend to contaminate the cooled powder charge. If the powder body is prepared without the addition of carbon to the original powder mixture charge of zirconium and boron, the hydrogen may be shut off at the completion of the 1800° C. heating cycle described above, and a graphite block is placed over the exhaust. The powder charge in the crucible will then cool within a carbonaceous atmosphere generated by the graphite crucible and the excess boron of the

charge will combine with the carbon of the carbonaceous atmosphere within the crucible into boron containing 4 to 33 atomic percent carbon in solid solution.

At the end of the cooling cycle, the powder charge in the crucible will form a lumpy semi-powdery body which is readily removed from the graphite crucible and pulverized by a simple crushing procedure. Iron or steel jaws or like crushers should not be used for this pulverization step since the powder body should be protected against very harmful contamination with iron. The crushed powder then is subjected to further comminution into a fine powder of a particle size such as between 2 and 8 microns average particle size. A gaseous-type vortex pulverizing equipment of the type described hereinbefore has been found satisfactory for this purpose. By way of example, on chemical analysis, a body produced in the manner described above contained about 75% zirconium, 23% boron and 1 to 1.2% carbon, the body consisting principally of zirconium diboride  $ZrB_2$  with 4% of excess boron containing in solid solution an excess of 4 atomic percent carbon. In producing zirconium diboride  $ZrB_2$  powder with the desired excess of 2 to 7% carbon-containing boron, approximately 2% boron is usually lost through oxidation and this factor should be taken into account and compensated for in proportioning the original mixture of the ingredients of the zirconium and boron ingredients which are subjected to the treatment described above. Thus, in producing a powder body of  $ZrB_2$  containing 5% of carbon-containing boron in excess of the zirconium diboride  $ZrB_2$ , the original mixture of the powder ingredients subjected to the treatment described above, should be calculated to contain about 2 to 8% excess boron over the amount required to yield the desired proportion of zirconium diboride  $ZrB_2$ .

In producing the powder mixture of  $ZrB_2$  with 2 to 7% of carbon containing excess boron, it is important that the mixture shall not contain any uncombined carbon in excess of about 1.5%, and this applies also to the cemented bodies made of such powder mixtures. If the cemented zirconium diboride  $ZrB_2$  material of the invention contains—in addition to the excess of 2 to 7% boron having in solid solution therein 4 to 33 atomic percent carbon—more than 1.5% uncombined or free carbon, the strength of the material is substantially reduced, and for best results, the uncombined carbon should be less than 0.5% of the material, and such material may be readily produced by the processes herein described.

#### Production of cemented zirconium diboride bodies

As explained above, shaped cemented bodies of zirconium diboride  $ZrB_2$  particles bound with 2 to 7% of excess boron containing carbon in solid solution, may be produced by the use of powder metallurgy or ceramic techniques. These techniques include hot pressing, cold pressing and sintering, extrusion and sintering, slip casting and sintering, and any combination of these techniques with intermediate presintering and machining operations.

Because of the unusually high stability of zirconium diboride  $ZrB_2$  mixed with 2 to 7% of carbon containing excess boron this powder body will not be detrimentally affected by contact with carbon when forming it into the desired shape by hot pressing in a graphite die. In such hot pressing procedure, the die may be heated either by direct current conduction, by resistance heating or by induction heating. As explained above, hot pressing in graphite die may be carried on with a pressure of about 3 to 4 t.s.i. If the powder body is hot pressed in a die formed of cemented zirconium diboride  $ZrB_2$  bonded with 2 to 7% of carbon-containing boron, pressures of 10 to 12 t.s.i. and higher may be applied to the die. In general, pressing with pressures of at least about 2 t.s.i. at temperatures of at least about 2000° C. are required for producing bodies of the desirable high

strength, heat shock resistance and corrosion-resistance at elevated temperatures.

It is of advantage to carry on the hot pressing process with induction heating because the pressed powder body may be brought to the desired temperature of about 2200 to 2700° C. in a very short time so that the die will have a slightly lower temperature than the heated powder mixture.

By way of example, the graphite die is heated by induction for a very short period when producing rocket nozzles weighing 15 pounds out of a powder body containing zirconium diboride with an excess of 5% carbon-containing boron which is subjected to a pressure of 3 t.s.i. within the graphite die in a very short period.

A similar zirconium diboride powder mixture was used for making fuel nozzles by pressing the powder body hydrostatically in a rubber die within a pressure of 10 to 25 t.s.i. The green compact was then presintered at an elevated temperature between 1200° and 1500° C. The presintered shaped compact was thereafter further shaped and machined to size with ordinary machine shop equipment, the compact having been linearly oversized by about 16% to compensate for shrinkage in the final sintering operation. After shaping, the presintered compact was subjected to the final sintering at a temperature between 2200 and 2700° C., thereby giving it ultimate density and strength.

Cemented bodies produced by hot pressing in the manner described above and consisting of zirconium diboride  $ZrB_2$  bonded with 5% of excess boron containing 4 to 33 atomic percent carbon in solid solution had the following physical properties:

Melting point ..... 2500° C.-2600° C.  
 Density ..... 5.2 to 5.3 grams per cc.  
 (cubic centimeter).  
 Hardness ..... Rockwell A, 87 to 89.  
 Weight gain in air at 1100° C.  
 for 200 hours ..... About 8 to 15 milligrams  
 per square cm.

It had a stress-to-rupture life given in the table below:

| At Temperature | Under Stress,<br>p.s.i. | Hours<br>Until<br>Ruptured |
|----------------|-------------------------|----------------------------|
| 980° C.        | 13,000                  | 310 to 320                 |
| 980° C.        | 14,000                  | 300+                       |
| 980° C.        | 16,000                  | 300+                       |
| 980° C.        | 18,000                  | 80+                        |

According to the invention the exterior surface of such shaped body which is to be exposed to corroding atmospheres at elevated temperatures of 700° C. and higher, is provided with an exterior surface stratum consisting of chromium oxide, dichromium boride  $Cr_2B$ , and an excess of chromium. The present invention is based on the discovery that when the exposed surface of a shaped body formed of particles of  $ZrB_2$  bonded with a 2 to 7% carbon-containing boron, is provided with a adhering surface stratum of chromium about .001 to .020 inch in thickness, and thereafter treated at an elevated temperature between about 1200° and 2000° C., the boron in the underlying strata of the cemented zirconium diboride will diffuse into the adhering chromium coating and form with the chromium a new compound of dichromium boride,  $Cr_2B$ , with an excess of chromium which exhibits a much higher resistance to corrosion than the underlying cemented material.

A satisfactory method of applying a chromium layer to the boron-bonded zirconium boride nozzle or other article is by electroplating. Standard plating methods may be employed. The following is an example of a satisfactory plating process. The article to be plated is first cleaned, for instance, in a 10% aqueous solution of sodium hydroxide solution, and then washed in hot

water. The surface of the article is then reactivated as by dipping in dilute aqueous hydrochloric acid. In the meantime an aqueous bath containing chromic acid (calculated as  $CrO_3$ ) and sulfate ion in the ratio of approximately 100:1 (for example, a bath containing 350 g. of  $CrO_3$  and 3.5 g. of sulfate ions per liter) is heated to about 60° C. Good results are obtained by plating the cleaned article in this bath at a current density of 1 ampere per square inch. The zirconium diboride body is made the anode and chromium may be employed as the cathode. Such a bath will produce in approximately 30 minutes a coating of .0015 inch thickness and in approximately 180 minutes a coating thickness of 0.01 inch.

Too great a thickness of chromium plating may tend to peel off. Good results are obtained with chromium platings of .002 to .004 inch thickness. Coatings of such thickness when subsequently converted by the heat treatment to the surface stratum of chromium boride, plus chromium and chromium oxide have excellent adhering properties. The chromium oxide may comprise as much as 30% of the said stratum.

The plated product such as that produced by the above described process is then subjected to the heat treatment at between about 1200° C. to 2000° C., whereupon the boron of the product diffuses into the chromium coating and/or vice versa to convert a portion of said chromium into the dichromium boride,  $Cr_2B$ . The heat treatment is carried out in an oxidizing or an inert atmosphere of helium, argon or in vacuum, for example. Since a certain amount of chromium oxide is desired in the final product a carbonaceous or hydrogen atmosphere are not desirable since both carbon and hydrogen have a tendency to reduce chromium oxides.

Rocket nozzles made of the cemented zirconium diboride particles bonded with 2-7% carbon-containing boron containing 4-33 atomic percent of carbon as described in said copending application Serial No. 363,043, now abandoned, but without the chromium boride coating of this invention, gave outstanding performances when subjected to repeated firing tests. For example, tests were carried out at flame temperatures exceeding 2700° C. and chamber pressures of up to 4000 p.s.i.g. (pounds per square inch gauge) with a variety of propellant mixtures of the oxidizing or reducing type and also with solid propellants. The coated product of the present invention equals the performance of the uncoated product in every respect and in addition has a considerably longer life than the uncoated product of said copending application.

It will be apparent to those skilled in the art that the novel principles of the invention disclosed herein in connection with specific exemplifications thereof will suggest various other modifications and applications of the same. It is accordingly desired that the present invention shall not be limited to the specific exemplifications shown or described therein.

I claim:

1. A hard homogeneous body of high strength and corrosion-resistance at high temperatures, at least about 95% of said body consisting of cemented zirconium diboride, wherein particles of  $ZrB_2$  are bonded by a boron substance containing carbon in solid solution, said boron substance forming about 2 to 7% of said cemented zirconium diboride, said body being substantially free of uncombined carbon over 1.5% of said body, said body having a protective surface layer comprising dichromium boride  $Cr_2B$ , chromium oxide, and chromium on at least a portion of the surface area thereof.

2. A hard homogeneous body of high strength and corrosion-resistance at high temperatures, at least about 95% of said body consisting of cemented zirconium diboride, wherein particles of  $ZrB_2$  are bonded by a boron substance containing carbon in solid solution, said boron substance forming about 2 to 7% of said cemented zirconium diboride, said body being substantially free of

uncombined carbon over 1.5% of said body, said body having a protective surface layer comprising dichromium boride Cr<sub>2</sub>B, chromium oxide, and chromium on at least a portion of the surface area thereof, the said protective surface layer being less than 0.004" thick.

2,141,640  
2,364,108  
2,406,683  
2,497,041  
5 2,555,372  
2,651,496

Cooper ..... Dec. 27, 1938  
Swentzel ..... Dec. 5, 1944  
Hensel et al. ..... Aug. 27, 1946  
Bodger ..... Feb. 7, 1950  
Ramage ..... June 5, 1951  
Buckland et al. ..... Sept. 8, 1953

References Cited in the file of this patent

UNITED STATES PATENTS

|           |             |               |    |
|-----------|-------------|---------------|----|
| 1,803,189 | Hoyt        | Apr. 28, 1931 | 10 |
| 1,853,369 | Marshall    | Apr. 12, 1932 |    |
| 2,088,838 | Cole et al. | Aug. 3, 1937  |    |
| 2,116,399 | Marth       | May 3, 1938   |    |

OTHER REFERENCES

Goetzel: "The Iron Age" (April 29, 1948), pp. 78-81.  
Glaser: Trans. AIME (April 1952), Journal of Metals, pp. 391-396.